

## UNITED STATES PATENT OFFICE

RAFAEL GUASTAVINO, OF BAY SHORE, NEW YORK, ASSIGNOR TO R. GUASTAVINO COMPANY, OF NEW YORK, N. Y., A CORPORATION OF MASSACHUSETTS

## ACOUSTICAL PRODUCT

No Drawing.

Application filed January 17, 1929. Serial No. 333,246.

This invention relates to acoustical structural material suitable for finishing or facing walls and ceilings in auditoriums and the like and having a high acoustical value possessing the property of absorbing sound waves ranging at least between C—1 and C—7 of the musical pitch. Primarily the material of the present invention is a material possessing the acoustical characteristics specified and of special utility, not only for the walls and ceilings of auditoriums and like places to prevent excessive reverberations and echoes, and the injurious focusing of sound, but also particularly available as a practical form of acoustical material suitable for hospitals and places where the sound absorbing feature is desirable, as well as the feature of being washable for cleansing without in any way affecting the character of the material or its coloring.

Another general object of the invention is to provide an acoustical product, preferably used in tile or block form which has a high porosity and can be made in various permanent colors and which also has the desirable quality of not being susceptible of shrinkage and also not affected by moisture and light.

Another separate and distinctive object of the invention is to provide a novel method of processing or making acoustical material which permits of the use of non-absorbent stony aggregate in combination with metallic coloring elements whose color is developed by the firing of the material, thus obtaining an acoustical structure or material wherein the colors are set and made permanent by the firing and will not be affected in any way by the exposure or use of the same; also contributing to that important phase of the invention which provides for an acoustical tile or block which may be used in the construction of high-grade masonry forming the permanent interior finish of a wall or ceiling.

The present invention differs materially from acoustical material of a ceramic nature such as that disclosed in my former Patent No. 1,119,543 granted December 1, 1914, wherein the porosity in the final product is the result of burning out of vegetable or

organic material originally mixed with the raw clay to provide the inter-communicating pores throughout the mass, and also from that type of non-ceramic acoustical material covered by the joint patent of Sabine & Guastavino Reissue No. 14,992, granted November 23, 1920, wherein the particles of body material, which are preferably graded, are merely bonded to each other at the points of contact with such a binder, as for example, Portland cement. The methods of these former patents for producing an acoustical finishing material represent the art as known to the applicant and differ from the present invention, which contemplates an acoustical or sound absorbing material consisting of particles of graded body material bonded to each other at their points of contact by a flux which becomes the binder upon the firing of the material and produces a material of glassy character throughout which is easily washed or cleansed.

Accordingly, in carrying forward the present invention there is used preferably a graded stony or vitrified ceramic aggregate having incorporated, in a mixture therewith, a flux, or which involves a fluxing element, which, upon the final firing of the material will fuse and permanently bind the aggregate particles together at their points of contact which forms the product with inter-communicating pores throughout which extend to the surface and which are of such size as to best absorb sound waves ranging, for example, between C—1 and C—7 of the musical pitch.

In its concrete aspect the invention consists of an aggregate of preferably graded stony or ceramic particles, including a fluxing element and preliminarily molded into the desired tile or block form with a shape maintaining element which may be the flux itself or a separate substance, such as an organic or inorganic adhesive. Subsequently, after the tile or block has been shaped to form, such form is then subjected to a firing heat thereby to flux together the particles only at their points of contact, and at the same time developing, setting, and

making permanent, any color which it is desired to give to the material.

More specifically it may be said that the invention is carried into effect by using a 5 preferably graded aggregate composed of quartz, feldspar, sand, or any practical selection of vitrified particles, such as glass, which have been ground and screened to a proper grading. This aggregate preferably 10 has mixed with it a certain proportion of a flux, such for example, as boracic acid, borax, lime, oxide or carbonate of lead, or any other suitable flux or combination of fluxes so that when the mixture is worked up and dampened the same may be molded in suitable 15 forms for the making of tiles, bricks, slabs or blocks. The material thus molded or cast is preferably formed in a mold having a steel plate at the bottom so that after the pressing 20 of the material into the mold, and thereby shaping it, the same may be left on the plate to be properly dried under suitable atmospheric conditions for a period of usually 25 approximately three or four days. When thus dried the shaped acoustical material is 30 placed in a suitable kiln or oven and fired at a temperature ranging from approximately 1500° to 2000° Fahrenheit so that the fluxing element, included in the aggregate, 35 will fuse and bind the aggregate particles together at the points of contact only, thereby leaving intercommunicating pores throughout the body of the material and also extending to and through the surface 40 thereof as previously indicated.

It will be understood that in the very nature of some of the particles used, a separate fluxing element may be omitted, as for example, glass alone will act as its own flux 45 by carrying the temperature to the proper degree or it may be mixed with a flux as already referred to, and feldspar is another example of a material used that will operate as its own flux at a high temperature. 50 When material of this kind is used, acting as its own flux, the mixed aggregate is held and maintained in its preliminary molded shape by a separate shape maintaining element, such as an organic or inorganic adhesive, so that it will therefore be understood 55 that, in carrying out the invention, while a separate fluxing element is preferably employed as part of the mixture, nevertheless, an aggregate material made up of a substance which in itself acts as a fluxing element may be made to serve the purposes of the invention.

It will now be seen that a distinguishing 60 feature of the present invention is that the acoustical product resulting from the foregoing method of processing will have sufficient stability, before firing, to permit of

stenciling of designs thereon, so that the design may be "fired in" the final product and that an important phase of the invention is that the process of making the material lends itself to the use of a metallic coloring element whose color is developed by the firing of the material and is thereby set and made permanent. Another feature of importance to note in connection with the invention is that the firing of the preliminarily shaped 70 product to the fluxing temperature will cause the material to become of a vitreous or glassy characteristic and impervious to moisture, while at the same time being made readily 75 cleansable or washable as hereinbefore referred to.

Another phase of the invention that should be noted is that in some cases it may be desirable to associate with the aggregate material not only a separate flux, as for instance, boracic acid, but also Portland cement. The importance and advantages of this combination is that the Portland cement acts not only as an hardening agent and binder but at a high temperature also acts as a flux. This will make an acoustical material which can be readily molded and set to the desired shape and after firing will possess extreme rigidity, strength and permanence.

From the foregoing it is thought that the structural and process features of the present invention will now be readily appreciated without further description and it is understood that changes in material and in process may be resorted to without departing from the spirit or sacrificing any of the advantages of the invention.

I claim:

1. A tile or block consisting of graded non-absorbent silicious aggregates of a character that are superficially fusible with or without a flux at a temperature between 1500° to 2000° F. and of a size to provide a porous mass capable of absorbing sound between C-1 and C-7 of the musical pitch, bonded at their points of contact by superficial fusion.

2. An acoustical tile or block providing a porous vitreous exposed outer face and consisting of graded non-absorbent siliceous aggregates of a character that are superficially fusible with or without a flux, said graded aggregates being of a size to provide a porous mass capable of absorbing sound between C-1 and C-7 of the musical pitch and bonded at their points of contact by superficial fusion.

In testimony whereof I hereunto affix my signature.

RAFAEL GUASTAVINO.